

## UNITED STATES PATENT OFFICE

2,404,463

## AQUEOUS EMULSION PAINT

Marvin T. Schmidt, Chicago, Ill., assignor to  
United States Gypsum Company, Chicago, Ill.,  
a corporation of Illinois

No Drawing. Application February 23, 1944,  
Serial No. 523,581

11 Claims. (Cl. 106—143)

1

This invention relates to an improvement in the art of manufacturing colored washable emulsion paints sometimes referred to as resin emulsion paints and more particularly to a paint which is uniform in color and free from streaking and blotching when applied to ordinary surfaces.

It is the purpose of this invention to produce a colored emulsion paint which is substantially free from blotching and streaking when applied in thin film form, particularly to surfaces which are high in absorption such as plasterboard or a lime putty finish.

It is well known that colored emulsion paints, such as those made using alkyd resins, as well as other film forming materials, will sometimes show differences in color when applied over surfaces exhibiting different degrees of "suction" in various areas, though the paint itself is uniform; and in addition, these paints often show differences of color as streaks along the path of the brush when the paint is applied over such surfaces. When a painted surface exhibits either brush streaks or blotches a very undesirable condition exists which is a consistent cause for complaint in the field. Unfortunately, repainting the non-uniform colored surface does not always result in an improvement of the surface, but in many cases magnifies the difficulty. The exact cause of these conditions is not known but it is believed due to irregular absorption of the surface.

In the description of this invention the term "blotching" is defined to mean the variation in shade in localized areas different from the field color when the same shade of paint is used throughout, and where such difference is not accountable for by a corresponding difference in color of the surface being painted. Also, by the term "streaking" is meant the color variation which follows the path of the brush strokes in parallel lines like the ridges and depressions following the brush though there may not be such ridges and depressions.

This difficulty of streaking and blotching can be overcome by first thoroughly sealing or priming the surface with a varnish type of surfacing material. This treatment is expensive when applied only for this purpose as in general it is not ordinarily needed to accomplish any other purpose. In fact, many of the walls to which an emulsion paint is to be applied are "green" and

2

hence cannot be properly sized until dry. One of the outstanding advantages of an aqueous emulsion paint is that it can be applied to green walls without previous drying, and to dry and size the wall so that it can be painted would be doing away with one of the big advantages in using this type of paint.

It has been discovered that by the simple addition of certain materials this difficulty of streaking and blotching can be practically completely eliminated. Thus if difficulty of this type is encountered in actual field application, it can be overcome merely by mixing a small quantity of the inhibiting material into the paint.

15 The materials that accomplish the purpose of this invention were obtained as a result of a great number of trials using various types of materials. No predictions arising out of knowledge commonly known to those skilled in the art could be made. 20 No explanations can be made as to why only certain few materials will work satisfactorily while a great range of other materials will not. Numerous theories were considered, but no data to support them could be evolved.

25 Only a very limited number of materials can be used for the purpose. One class of materials which has been found satisfactory is the fatty acid esters of polyethylene glycols, such as the type known as and sold under the trade name

30 of "Carbowax 4000" and manufactured by the Carbide and Carbon Company. It has been found that the esters of saturated or unsaturated fatty acids of between 12-24, inclusive, carbon atoms, particularly stearic, formed with a polyethylene glycol such as "Carbowax 4000," as referred to above, are very well suited for carrying out this invention. Other materials which prevent streaking and blotching form the subject of another application, Serial No. 523,580, filed February 23, 1944.

35 In carrying out this invention, it is preferred to add the material to the paint during its formulation as a more complete and accurate intermixing can be accomplished; though it is within the scope 40 of this invention, and sometimes necessary, to add the polyethylene glycol ester to the paint in the field. For purpose of illustrating the preferred method of carrying out this invention in the following example, the material will be added during 45 formulation.

The forthcoming example clearly describes a paint composition which but for the inhibiting material incorporated therewith will result in pronounced streaking and blotching when applied to many types of surfaces.

| Emulsion                     |        | Pounds |
|------------------------------|--------|--------|
| Ester gum-linseed oil binder | 166    |        |
| 6% cobalt drier              | 8      |        |
| Casein solution, 20% solids  | 340    |        |
| Paste paint                  |        |        |
| Emulsion                     | 514.0  |        |
| Phthalocyanine blue          | 31.6   |        |
| Cadmium yellow               | 31.6   |        |
| Bone black                   | 4.75   |        |
| Titanium dioxide             | 900    |        |
| Fine mica                    | 60     |        |
| Pine oil                     | 25     |        |
| Water approx                 | 350    |        |
| Carbowax ester 25% solids    | 35-280 |        |

The ester gum-linseed oil binder is prepared by heating to a temperature of 580 degrees F. for about one hour, 41.5 lbs. of ester gum with 124.5 lbs. of heat bodied linseed oil. The cobalt drier is then added. The drier can be of the naphthenate type. This mixture, while in liquid form, is emulsified, by any of the well known methods of preparing an emulsion, with the casein solution to form a binder. Most any type of casein solution can be used. A suitable casein solution is one which is described in U. S. Patent No. 2,154,362. This can be used to advantage as it is stable for a considerable length of time to deterioration due to aging. However, the preparation of casein or other protein solutions using alkalies such as borax for use in emulsion paints is well established in the art and a detailed description of a procedure for making them need not be included in the description of this invention.

For the sake of convenience for those who may not be familiar with this art and with U. S. Patent No. 2,154,362, the following procedure, which is based upon the above patent can be used in preparing a casein solution. Following this patent the casein solution can be prepared by mixing 55 lbs. of commercial casein with 24 gallons of water with thorough stirring for a sufficient length of time until a smooth mixture of thoroughly soaked casein results. About 3 pounds and 6½ ounces of sodium stannate are dissolved in about 3½ gallons of water, while in a separate container about 10 lbs. of borax are likewise dissolved in about 2½ gallons of hot water. The sodium stannate solution is then added to the casein mixture, with constant agitation, and as soon as all of it has been added, the borax solution is then run into the mixture. An additional amount of, say, 3 gallons of water may then be added and the mixing continued while heating the mixture gradually to about 150 to 160 degrees F. or higher. The mixing is continued at the desired temperature until a smooth solution results. Using the proportion above given, the solution will be found to exhibit an alkaline reaction equivalent to from about pH 8.0 to pH 9.0. The ratio of casein to sodium stannate in the above formula is substantially 100:6.2. The sodium stannate used has the following formula:  $Na_2SnO_3 \cdot 3H_2O$ . While casein is the preferred type of protein, other proteins may be used including those derived from vegetable sources, for example alpha protein derived from soya beans.

When the emulsion has been prepared, using

additional water if necessary, the dry pigments and other ingredients are added and mixed in a suitable type of mixer. The Carbowax stearate is preferably added last.

The Carbowax stearate can be made by reacting polyethylene glycol, i. e., Carbowax 4000, with stearic acid or it can be purchased already prepared from the Carbide and Carbon Chemicals Corp., as well as other sources. It is preferred to add this material as a water paste, and containing about 25% of the solid material. This is prepared by heating 25 parts of the Carbowax stearate in 75 parts of water. Various modifications of the Carbowax, such as Carbowax 1500, can be used as well as equivalent materials sold under different trade names. Any of the polyethylene glycols can be used as long as the properties are such as to accomplish substantially the same results as with Carbowax 4000. It is not intended to limit this application to the addition of the stearate in paste form to the paint already prepared for it may be added in any manner and at any time during the formulation or use of the paint as long as the effective result of this material is obtained.

Neither is it the intention to limit the scope of this invention to a neutral ester of a fatty acid; for the polyethylene glycol need not all be esterified, though a mere solution of the glycol in the fatty type of acid is not enough. The mixture must be heated to effect some type of reaction between the two which need not be an entirely pure ester in itself. There can be an excess of the acid over that of the polyethylene glycol and excellent results will still be obtained. Hence, throughout the specifications and claims of this invention the word "ester" is intended to mean a mixture of a fatty acid and a polyethylene glycol solution, in stoichiometrical quantities or otherwise, which has been heated or treated to effect a reaction between a portion or all of the constituents. Also it is not necessary that the ester be prepared from the acid alone for other esters can be used, such as the glyceride as long as the fatty acid radical can be made to react with the polyethylene glycol in same manner. In other words, an ester interchange can be used to prepare the polyethylene glycol ester if desired as well as other methods.

After the Carbowax stearate paste has been added and the mixing operation has been completed, the paste is then passed through a roller mill to insure complete dispersion of the pigments into the vehicle and to form a paint completely free from lumps.

Various types of pigments, fillers and other finely divided inorganic material can be used in the preparation of paints which can be benefited by this invention. However, it is necessary that some coloring material be present as streaking and blotching have not been observed to any great extent in white paints. Since water is the thinner, it is possible to use a wide variety of low index of refraction materials such as clays, mica, etc., known in the trade as filler or extenders to replace a certain amount of the more expensive higher index of refraction materials known as pigments, such as lithopone and titanium dioxide, as required in an oil type of paint. Since both types of material can be used, in order to define these two types of material generically, the word "pigment-fillers" will be used in the forthcoming claims.

Paint prepared in the above manner will not exhibit the streaking and blotching effects com-

monly associated with washable emulsion paints. This is done without any sacrifice in the desirable properties of this type of material and with only a slight increase in cost.

If the paint has already been prepared and it is desired to prevent streaking and blotching, then about 4 to 32 ounces of the 25% Carbowax stearate ester paste, mentioned above, can be added per gallon. Other esters of polyethylene glycol can be also used. Also it is not necessary that the ester be added in paste form. It may be expedient in many cases not to add the inhibiting material until actual trouble is experienced as the difficulty is only occasionally encountered.

Examples of the saturated and unsaturated fatty acids besides stearic between 12 and 24 carbon atoms inclusive which can be used in forming an ester with polyethylene glycol, such as Carbowax stearate 4000 to accomplish the purpose of this invention are myristic, palmitic, elaeostearic, dehydrated castor oil fatty acids, oleic, linolenic and linoleic. Other acids in this group will readily occur to those skilled in the art in which this invention is a part. The pure acids need not be used as the naturally occurring mixed acids are just as effective. In most cases the ester can be prepared by simply heating the polyethylene glycol with the fatty acid. In some cases it may be desirable to add an excess of the acid.

In the above example a mixture of ester gum and heat bodied linseed oil is used. It is not the intention to limit this invention to any of the ingredients used in the preferred embodiment set forth, for any water resistant film forming substance which will have utility in a colored emulsion paint may be used. It is not necessary that the material be a resin, though most of the emulsion paints in common use contain a resinous or polymerizable material, usually oleoresinous. Examples of some of the materials which can be incorporated are: treated or untreated oils having drying properties, alkyd resin, phenol formaldehyde resins, the various esters of rosin, synthetic and natural resins, such as congo gum, copal gum and manila gum. These can be used alone, in combination or with solvents; the particular manner in which they are used as well as the addition of other materials such as driers and the like are all within the skill of the art of which this invention is a part and need not be further described.

While it is preferred to use casein or some other protein material, such as Alpha protein derived from soya beans, as the emulsifying agent, it is not the intention to limit this invention thereby, for other emulsifying agents which are compatible can be employed. The volatile alkali soaps are especially suitable for the purpose.

It will be found that paints prepared in accordance with the principle set forth in this invention can be applied over practically any surface without danger of forming an appreciable amount of streaks or blotches. A uniform coloration will be obtained. Water paints applied over a lime putty finish and over wallboard are particularly liable to give trouble, yet no difficulty will be encountered if the paint is prepared following the principles set forth in this invention.

By way of summary this invention pertains to the prevention of color blotching or streaking in a colored aqueous emulsion paint by incorporating therein a polyethylene glycol ester of fatty acids from 12 to 24, inclusive, carbon atoms. The non-aqueous vehicle may consist of oils, var-

nishes, natural and synthetic resins, or other water insoluble film forming materials; these are preferably emulsified by the use of casein or similar materials.

Although there has been disclosed a practical embodiment of this invention and specific examples and uses, which are given to insure a clear understanding of the essence of this invention, it is not the intention to be limited thereby for obviously many variations may be made by those skilled in the art and still be within the scope of this invention which is only limited in extent by the forthcoming claims.

It is claimed:

1. A non-streaking, non-blotching, aqueous emulsion paint comprising a protein selected from the group consisting of casein and an alkali dispersible vegetable protein derived from soybean, a solvent for said protein, water, a water insoluble film forming material, colored pigment, and a streaking and blotching inhibiting material comprising an ester formed from the reaction of a polyethylene glycol and a fatty acid of from 12 to 24 carbon atoms per molecule.
2. A non-streaking, non-blotching, aqueous emulsion paint comprising a protein selected from the group consisting of casein and an alkali dispersible vegetable protein derived from soybean, a solvent for said protein, water, a water insoluble film forming material, pigment-filters, at least one of which is colored, and a streaking and blotching inhibiting material comprising an ester formed from the reaction of a polyethylene glycol and saturated and unsaturated fatty acids of from 12 to 24 carbon atoms per molecule.
3. The composition of claim 1 in which said water insoluble film forming material is capable of drying by oxidation and polymerization.
4. The composition of claim 1 in which said water insoluble film forming material is a resinous material selected from the group consisting of synthetic resins and natural resins, and a solvent for said resin.
5. The composition of claim 1 in which said water insoluble film forming material is an ester of resin acids.
6. An aqueous resin emulsion paint substantially free from streaking and blotching, comprising a water insoluble film forming material, colored pigment, an emulsifying agent, water, and a streaking and blotching inhibiting material comprising an ester formed from the reaction of a polyethylene glycol and saturated and unsaturated fatty acids of from 12 to 24 inclusive carbon atoms per molecule.
7. A non-streaking, non-blotching, colored, aqueous emulsion paint comprising a protein selected from the group consisting of casein and an alkali dispersible vegetable protein derived from soybean, a solvent for said protein, water, a water insoluble film forming material, pigment-filters, at least one of which is colored, and an ester formed from the reaction of stearic acid and a polyethylene glycol.
8. A non-streaking, non-blotching, aqueous emulsion paint comprising a protein selected from the group consisting of casein and an alkali dispersible vegetable protein derived from soybean, a solvent for said protein, water, pigment-filters, at least one of which is colored, a water insoluble film forming material and from about 1 to about 8 ounces of an ester, formed from the reaction of a polyethylene glycol and a fatty acid containing from 12 to 24, inclusive, carbon atoms

per molecule, to each gallon of said aqueous emulsion paint.

9. A non-streaking, non-blotching, aqueous emulsion paint comprising casein, a solvent for said casein, a water insoluble film forming oleoresinous material containing an alkyd resin, pigment-fillers, at least one of which is colored, and an ester formed by the reaction of polyethylene glycol and a fatty acid selected from the group consisting of stearic, palmitic and oleic acids.

10. An aqueous emulsion paint substantially free from streaking and blotching comprising a water insoluble film forming oleoresinous binder comprising the resulting product formed by heating an oil capable of drying by oxidation and polymerization with a resin selected from the group consisting of synthetic resins and natural resins, a volatile alkali soap emulsifying agent, water, pigment-fillers, at least one of which is colored, and the ester formed by heating a mix-

5  
10  
15

20

ture of polyethylene glycol and a saturated and unsaturated fatty acid containing from 12 to 24 inclusive carbon atoms per molecule.

11. An aqueous emulsion paint substantially free from streaking and blotching comprising a protein selected from the group consisting of casein and an alkali dispersible vegetable protein derived from soya beans, a solvent for said protein, a water insoluble film forming resinous binder comprising the resulting product formed by heating an oil capable of drying by oxidation and polymerization with a resin selected from the group consisting of synthetic resins and natural resins, water, pigment-fillers at least one of which is colored, and the ester formed by heating a mixture of a polyethylene glycol and a fatty acid containing from 12 to 24 carbon atoms per molecule.

MARVIN T. SCHMIDT.